

March 17, 1942.

H. D. HOLLER

2,276,973

INSULATED ELECTRIC HEATER AND METHOD OF MAKING THE SAME

Filed Sept. 15, 1939



Fig. 1.



Fig. 2.

WITNESSES:

*E. J. Oberheim*  
*James W. Ely*

INVENTOR

*Homer D. Holler.*  
BY  
*Frank Savage*  
ATTORNEY

## UNITED STATES PATENT OFFICE

2,276,973

INSULATED ELECTRIC HEATER AND  
METHOD OF MAKING THE SAME

Homer D. Holler, Export, Pa., assignor to Westinghouse Electric &amp; Manufacturing Company, East Pittsburgh, Pa., a corporation of Pennsylvania

Application September 15, 1939, Serial No. 295,053

7 Claims. (Cl. 201—64)

This invention relates to insulated electric heaters and to the method of insulating such heaters.

In producing insulated electric heaters, it has been found to be difficult to provide an insulation of uniform homogeneous composition which is capable of withstanding the high temperatures sometimes encountered in service while having the characteristic of being non-corrosive. It has also been difficult to insulate the heater elements, the existing methods requiring considerable care in practicing the steps thereof, while the results are not always uniform.

An object of this invention is the provision of an insulated electric heater unit, the insulation of which is a dense homogeneous mixture of materials which are non-corrosive and have high electrical resistivity.

A further object of this invention is the provision of a method of insulating electric resistor wires of the heater type, whereby a hard, dense, non-corrosive insulating coating is formed about the wire.

Other objects of this invention will become apparent from the following description when taken in conjunction with the accompanying drawing, in which

Figure 1 is a side view of a resistor element embodying the teachings of this invention; and

Fig. 2 is an enlarged view in section of the element of Fig. 1, taken along the line II—II.

In practicing this invention, any of the well-known metallic resistor units may be employed, and particularly the metallic heating wires 10, as illustrated in the drawing, such as are utilized in the heating units of electric roasters, strip heaters, hot plates and the like. All of these elements should be so insulated as to prevent oxidation thereof and to electrically insulate them from the apparatus in which they are employed, while permitting the heat developed therein to flow therefrom.

In order to satisfactorily insulate such heating wires, this invention provides for utilizing the reaction products of a mixture of materials as the insulating material 12 for embedding the heating wire 10 therein as illustrated in the drawing. The materials employed for forming the insulating material comprise a mixture of magnesium oxide and ammonium borate. In 50 making the mixture for applying to the wire to be insulated, the magnesium oxide and the ammonium borate are thoroughly mixed, with the ammonium borate constituting from 25% to 50% by weight of the mixture, after which sufficient

water is added to the resulting mixture to give it a creamy, mud-like consistency so that it can be poured. The amount of water employed to give the mud-like consistency to the mixture will vary 5 depending upon the grade of magnesium oxide employed, but in all cases should be so limited to that quantity which gives the mud-like consistency to the mixture. Where an extremely pure grade of magnesium oxide is utilized, it is preferred to make the mixture in a 1:1 ratio by weight of magnesium oxide and ammonium borate. For the impure grades of magnesium oxide, smaller quantities within the range of 25% to 50% by weight of the ammonium borate can be employed giving a mixture having a ratio ranging between 1:1 and 2:1 by weight of the magnesium oxide to the ammonium borate.

With the magnesium oxide and ammonium borate formed into the mixture having a mud-like consistency, it is applied to the wire to be insulated in any of the well known manners for completely embedding the wire. Thus the mixture can either be poured directly about the wire or it can be extruded about the wire, or films of the mixture can be applied to both sides of a heating element to envelop it. Regardless of the method employed for enveloping or embedding the heating wire in the mixture of magnesium oxide and ammonium borate, it is found that where the mixture, as applied, has a mud-like consistency it will set about the heating wire or unit in a manner similar to the setting of plaster of Paris. In this form, the embedded heating wire can be moved without danger to the applied coating.

In order to produce the finished insulating coating about the wire, the embedded article is placed in any suitable furnace and subjected to a baking treatment at a temperature of not less than 120° C., and preferably between 120° C. and 180° C., it being found that such baking effects a reaction upon the components of the mixture constituting the coating. This reaction between the magnesium oxide and ammonium borate is accompanied by the evolution of ammonia and moisture from the mixture, and gives a resulting product comprising a uniform, intimate and homogeneous mixture of magnesium oxide and magnesium borate.

In a particular embodiment of this invention, a material which is inert with respect to the reaction between the magnesium oxide and ammonium borate is included in the mixture to add strength to the resulting insulating coating and to reduce the cost per pound for insulation. Pot-

ter's flint is quite satisfactory for this purpose when added to the mixture in an amount ranging up to about 50% of the total mixture with the magnesium oxide and ammonium borate constituting the balance. In this particular mixture the ammonium borate forms from about 35% to 50% by weight of the balance of the mixture. In all cases the magnesium oxide and ammonium borate are employed in the ratio ranging between 1:1 and 2:1 of magnesium oxide to ammonium borate whether or not the potter's flint is present in the mixture. A particularly good insulation is found to be formed where the ammonium borate, magnesium oxide and potter's flint are employed in a 1:2:3 ratio.

When the flint, magnesium oxide and ammonium borate is mixed with water to have a mud-like consistency and applied to the wire and treated in the manner hereinbefore described, it is found that the flint takes no part in the chemical reaction between the magnesium oxide and ammonium borate but remains in the resulting insulating coating, uniformly distributed therein and aids in giving added strength to the reaction products of the magnesium oxide and ammonium borate, the resulting insulating coating consisting of a uniform, intimate and homogeneous mixture of flint, magnesium oxide and magnesium borate.

Upon examination, it is found that the insulating coating comprising the uniform and homogeneous mixture of magnesium oxide and magnesium borate, either by itself or with the potter's flint as hereinbefore described, is quite dense and extremely hard. Further, it is found that the resulting reaction product has good thermal conductivity, an extremely high electrical resistivity and the desired characteristic of being non-corrosive. In addition to the foregoing desired characteristics, the insulation will not crack when subjected to the extreme changes in temperature as are encountered in operating the formed unit as a heating element, nor is it affected by the humidity of the atmosphere in which it is operated, the insulating coating being free of decrepitation.

Although this invention has been described with reference to a particular embodiment thereof, it is, of course, not to be limited thereto except insofar as is necessitated by the scope of the appended claims.

I claim as my invention:

1. The method of insulating electric resistor wires of the heater type comprising the steps of, embedding the wire in a mixture of magnesium oxide and ammonium borate having a ratio of between 1:1 and 2:1 and sufficient water to give the mixture a mud-like consistency, letting the mixture set in position about the wire, and heating the mixture while in position about the wire to effect a reaction between the magnesium oxide and ammonium borate whereby ammonia is evolved and a hard, dense, noncorrosive coating of intimately mixed magnesium oxide and magnesium borate is formed about the wire.

2. The method of insulating electric resistor

wires of the heater type comprising the steps of, embedding the wire in a mixture of magnesium oxide and ammonium borate having a ratio of between 1:1 and 2:1 and sufficient water to give the mixture a mud-like consistency, letting the mixture set in position about the wire, and heating the mixture while in position about the wire at a temperature of at least 120° C. to drive off the moisture therefrom and simultaneously to effect a reaction between the magnesium oxide and ammonium borate whereby ammonia is evolved and a hard, dense, non-corrosive coating of intimately mixed magnesium oxide and magnesium borate is formed about the wire.

3. An insulated electric heater comprising in combination, a resistor wire and a coating of insulating material disposed thereon, said coating comprising a hard, dense, non-corrosive material having a high electrical resistivity and comprising an intimate and homogeneous mixture of magnesium oxide and magnesium borate as essential binding elements thereof.

4. An insulated electric heater comprising in combination, a resistor wire and a coating of insulating material disposed thereon, said coating comprising an intimate and homogeneous mixture of magnesium oxide and magnesium borate formed by effecting a reaction between magnesium oxide and ammonium borate in the ratio of between 1:1 and 2:1, the coating being dense and non-corrosive.

5. An insulated electric heater comprising in combination, a resistor wire and a coating of insulating material disposed thereon, said coating comprising a hard, dense, non-corrosive material having a high electrical resistivity and consisting of an intimate and homogeneous mixture of potter's flint, magnesium oxide and magnesium borate, the magnesium oxide and magnesium borate being present as essential binding elements in the coating and binding the homogeneously distributed potter's flint.

6. An insulated electric heater comprising in combination, a resistor wire and a coating of insulating material disposed thereon, said coating comprising an intimate and homogeneous mixture of potter's flint, magnesium oxide and magnesium borate, the magnesium oxide and magnesium borate having been formed by effecting a reaction between magnesium oxide and ammonium borate in the ratio of between 1:1 and 2:1, the coating being dense and non-corrosive.

7. An insulated electric heater comprising in combination, a resistor wire and a coating of insulating material disposed thereon, said coating comprising an intimate and homogeneous mixture of potter's flint, magnesium oxide and magnesium borate, the magnesium oxide and magnesium borate having been formed by effecting a reaction between magnesium oxide and ammonium borate in the presence of the potter's flint, the ratio of the ammonium borate, magnesium oxide and potter's flint being 1:2:3, the coating being dense and non-corrosive.

HOMER D. HOLLER.